

March 24, 1970

G. SCHLEMON

3,501,857

GARMENT TREATMENT METHOD

Filed June 11, 1968

2 Sheets-Sheet 1



FIG. 1



FIG. 2

INVENTOR  
GEORGE SCHLEMON

BY

*Jones & Thomas*

ATTORNEYS

March 24, 1970

G. SCHLEMON

3,501,857

GARMENT TREATMENT METHOD

Filed June 11, 1968

2 Sheets-Sheet 2



FIG. 3

FIG. 4



INVENTOR  
GEORGE SCHLEMON

BY *Jones & Thomas*  
ATTORNEYS

1

3,501,857

**GARMENT TREATMENT METHOD**  
George Schlemon, 3060 Pharr Court NW,  
Atlanta, Ga. 30305

Continuation-in-part of application Ser. No. 676,098, Oct. 18, 1967, which is a continuation-in-part of application Ser. No. 543,996, Apr. 20, 1966. This application June 11, 1968, Ser. No. 736,176  
Int. Cl. D06f 71/00

U.S. Cl. 38—144

5 Claims

**ABSTRACT OF THE DISCLOSURE**

A method and apparatus for imparting a permanent press to garments comprising arranging the garments in their respective proper pressing position on a pressing surface, applying light pressure to the garments with a flexible screen which substantially conforms to the shape of the garments on the pressing surface, passing substantially saturated steam from the pressing surface through the garments and through the flexible screen to loosen the fabric of the garments, and passing air heated to a temperature at which the fabric is cured through the garment.

**CROSS REFERENCE TO RELATED APPLICATIONS**

This application is a continuation-in-part of application Ser. No. 676,098, filed Oct. 18, 1967, which was 30 a continuation-in-part of application Ser. No. 543,996, filed Apr. 20, 1966, now abandoned.

**BACKGROUND OF THE INVENTION**

Permanently pressed garments have been gaining wide commercial success of late due to the fact that the shape of the garment, as initially sewn and pressed, is locked in whereby the seams lie flat and neat, puckering is virtually eliminated, and the smooth, unblemished surface of the fabric is substantially retained for the life 40 of the garment.

At the present time there are generally four accepted procedures for obtaining permanently pressed garments, all of which are dependent upon the type of fabric used to form the garments. By type of fabric is meant the 45 pre-treatment of pre-conditioning given to the fabric, the type of weave, and the type of filaments used to make the fabric.

The first such procedure may be referred to as a post-cure system. In this procedure the fabrics are impregnated with chemical cross-linking finish as they are produced at the fabric mills. These chemical finishers are well known in the art and new ones are continuously being developed. The impregnated fabrics are then dried at low temperatures so that only a minimum of cross-linking occurs thereby rendering the fabrics "sensitized" but not cured. The "sensitized" fabrics are shipped to the garment manufacturers to be cut and sewn into garments. The thus formed garments are thereafter pressed into the desired shape and fully cured at elevated temperatures to retain the pressed garment shape. The curing operations are generally carried out in a batch placed in a continuous oven but would also be possible as a simultaneous aspect of the pressing operation, provided proper temperature conditions can be 65 achieved and maintained.

It is pointed out that chemical cross-linking finishes employed in the post-cured system react only with cellulosic fibers to produce the permanent press or set condition. Therefore, the fabrics employed therein must contain a sufficient cellulosic component, such as cotton or rayon for this procedure to be employed. Success-

2

ful application of this procedure has been had with polyester/cotton fabric of the 65/35 and 50/50 blend levels. It has also been successively applied to stretch denims having stretch nylon warp and cotton filling, as well as to stretch blends of polyester/cotton/spandex.

5 A second procedure for obtaining permanently pressed garments is sometimes referred to as the pre-cure system. In this procedure the fabrics are impregnated with a chemical cross-linking finish which reacts only with the cellulosic component of the fabrics just as in the post-cure system and, therefore, the fabrics must have a a cellulosic components. However, in this instance the fabrics must also contain a quantity of non-cellulosic thermoplastic fibers. The impregnated fabrics according 15 to this procedure are fully cured in the flat state at the mills. After the fully cured fabrics have been received and formed into garments at the garment manufacturing facilities the resulting garments are pressed with sufficient heat and pressure to permanently reshape the fabric and set the non-cellulosic thermoplastic fiber component in the proper shape for the garment. Fabrics which may be employed according to this pre-cure system include polyester/cotton blends and stretch blends of 75/25 cotton/nylon.

25 A third procedure, herein referred to as the re-cure system, may also be used to obtain permanently pressed garments and involves the use of a special chemical cross-linking reactant and a special catalyst. Again, these special chemicals only react with the cellulosic component of the fabric, as in the post cure and pre-cure systems, but the impregnated fabrics in this procedure are then substantially cured at the mills, i.e., up to 86% of the cross-linking reactions may have taken place. Upon being formed into garments, the fabrics are steam pressed whereby some of the previous cross-linking is broken or disrupted due to the presence of water. Subsequently, such cross-linking is reformed along with a complete cure by means of additional heat. Thus, in effect, the initial substantially cured fabric is temporarily uncured and then fully re-cured. The cellulosic component as well as the thermoplastic component, of the re-cured fabrics are both permanently shaped by the subsequent application of heat. The method and apparatus of the present invention is particularly suitable for this procedure in obtaining permanently pressed garments.

50 The last procedure for obtaining permanently pressed garments involves no chemical cross-linking reactant and, therefore, no curing, but rather depends entirely on the heat setting characteristics of thermoplastic fibers. Garments made from fabrics of this nature can be permanently pressed into shape according to this procedure at temperature of about 300° F. to 400° F. depending on the particular thermoplastic used. These temperatures may also vary to below 300° F. and above 400° F. Examples of fabrics that may be used in this procedure include blends of polyester/acrylic and polyester/nylon, or it may comprise 100% polyester.

55 While the above discussion has been mainly concerned with cellulosic and non-cellulosic thermoplastic fibers which may be heat-set, it is further pointed out that wool may also be permanently pressed. Since wool is a keratin material and possesses a natural memory it is necessary to treat the wool with a chemical reducing agent, such as monoethanolamine sulfite, whereby the natural memory is lost. Upon repressing the treated wool fabric with heat, a new memory may be created and thus the fabric is permanently pressed.

60 The permanent pressing with which the present method and apparatus are concerned relates to the above described procedures. Therefore, wherever the term "permanent press" is used hereinafter, it is intended to gen-

erally relate to these pressing procedures, as opposed to conventional pressing which is of a non-permanent nature. This is not meant to imply that the present method and apparatus cannot be used with conventional pressing as it is generally applicable to all types of pressing.

As is apparent from the above permanent press procedures the newly formed garments are in all cases subjected to pressing operations to provide the garment with its initial shape. In some instances the thus pressed garments are further subjected to a curing operation to obtain permanence of shape while in others the garments are permanently pressed as a result of the pressing operation alone. The pressing operations in all cases, however, must be controlled with respect to the temperature conditions so as to effect the desired cross-linking or curing when chemical finishes are employed or the desired heat-setting when non-cellulosic thermoplastic fabrics are employed.

The heretofore conventional pressing procedures and apparatus are not adequate for performing permanent press operations since the conventional apparatus does not control the temperatures and pressures necessary to obtain permanent pressing. By way of examples, these presses have generally comprised a pad covered buck and an uncovered metal head which is adapted to be raised and lowered into engagement with a garment placed on the buck. The head is usually provided with an upper chamber in which steam under pressure is stored and a lower chamber into which the steam from this upper chamber is released for dispersion through a plurality of holes or apertures in the lower pressing surface of the head. Often times, steam is additionally supplied to the buck which is then dispersed through the pad covering.

The storing of steam in the head and the repeated release of steam out of the head cause the pressing surface of the head and buck to become extremely hot and difficult to control. Moreover, because of the storing of high pressure steam, the heads have been massive and have required large and expensive structures to support, raise and lower them. As a result, garments being pressed according to permanent pressing procedures may very likely be exposed to uncontrolled excessive heat and pressure which may not only interfere with the permanent press of the garment but also may result in a "shine" on the garments. The shine created on a garment results from the nap of the fabric being crushed flat into the threads so that a flat reflective surface is created.

Not only do the conventional presses have disadvantages with respect to garments being permanently pressed but they also create hazardous conditions to the operator of the press. Since steam is applied from the head to the garment backed by the pad on the buck and before a drying vacuum is applied, these conventional pressing operations result in excess steam being freely spread about the region of the press. This is due to the fact that the steam supplied to the pressing surfaces has nowhere to escape except to the surrounding region of the press, particularly when steam is also supplied from the buck.

#### SUMMARY OF THE INVENTION

The present invention substantially eliminates these difficulties and limitations encountered with the previously existing methods and apparatus for permanently pressing garments. In accordance with the present invention, the massive steam containing head with its hazards to the operator and its excessive heat and pressure which tends to damage synthetic fabrics and blends and to "shine" the fabrics is eliminated. Moreover, the present invention provides for positive control over temperature conditions necessary to permanent pressing while maintaining low pressures on the garments and preventing "shine" by utilizing a steam cycle and a heated air cycle; that is, steam at a controlled temperature is passed

through the garment, and air heated to a prescribed temperature is passed through the garment.

The improvements of the present invention are achieved through the use of an improved head which is flexible, light, and inexpensive in construction, and an improved buck which includes a chamber communicating with its pad, a steam regulator, and an air heater. The head contains no stored steam nor does it supply any steam to the pressing surfaces of the press. Steam is supplied to the press solely through the buck whereupon it diffuses through the pad on the buck and into the garment spread thereover. The head provides a vacuum which withdraws the steam and heated air from the pressing surfaces as they pass through the garment and thereafter exhausts it from the press or recirculates it to the steam source for the buck. During normal operation of the apparatus, steam is passed through the garment as the garment is pressed between the head and buck, the steam cycle is terminated, and air heated to the temperature range proper for curing the garment is passed through the garment. The heated air cycle is employed after the garment has been initially steam pressed to produce the necessary curing or heat-setting in the garment for properly permanently pressing the material.

20 The head is fabricated of flexible material and a wire mesh or screen is stretched across its lower portion to form the garment engaging surface of the head. When the head is lowered into engagement with a garment on the buck, the head will flex to allow the screen to conform to the shape of the garment, and the raised or bulky portions of the garment will encounter approximately the same pressure or force from the head as the other portions of the garment. Thus, the bulky portions of the garment will protrude slightly into both the pad on the pressing buck and into the screen of the head.

25 Temperature control for permanent pressing according to the present invention is achieved by regulating the temperature of the heated air through heating means as are well known in the art, e.g., electrical, gas-fired, etc. The pressing surfaces are provided with proper temperature conditions by passage of the heated air through the steam pressed garment and withdrawal of the heated air through the vacuum system of the head. The vacuum system operates continuously so that the pressing surfaces and the head are prevented from over-heating and the various temperature ranges necessary to obtain a permanent press of the garments may be controllably obtained. Also, the continuous vacuum functions to exhaust any excess steam or heated air from the vicinity of the apparatus when the head has been disengaged from buck, thereby providing the advantage of no excess steam or hot air being free to spread about the region of the press which would cause uncomfortable conditions and possible hazard to the operator. Moreover, since the head is flexible, does not overheat, and has a "light-touch" on the garments, substantially no damage or "shine" will be produced on the fabric of the garment being permanently pressed, the nap of the garment will be lifted throughout virtually the entire garment, and the bulky and thin portions of the garment will be treated in equal fashion.

30 These and other features and advantages of the invention will be more clearly understood from the following detailed description and the accompanying drawing.

#### BRIEF DESCRIPTION OF THE DRAWING

35 FIGURE 1 is a schematic view of a press according to the present invention and shows the improved head and buck in section.

40 FIGURE 2 is a bottom perspective view of the buck.

45 FIGURE 3 is a cross-sectional view of the buck and related components.

50 FIGURES 4 and 5 are schematic showings of the manner in which the head engages a garment placed on the buck.

## DESCRIPTION OF THE PREFERRED EMBODIMENTS

It should be understood that the following detailed description and the accompanying drawing disclose a preferred embodiment of the present invention but neither the method nor the apparatus of the present invention are limited to the details disclosed since they may be embodied in equivalent forms.

Referring now more particularly to the drawing, in which like numerals represent like parts through the views, FIGURE 1 shows a press provided with a buck 1 having a chamber 2 and an upper plate 3. The upper plate 3 of the buck is provided with a plurality of openings or apertures 4 which allow air and steam to escape from the chamber 2 and pass upward into the garment being permanently pressed. A conventional pad comprising a cover cloth 5 and a porous resilient layer 6 coextensively cover the upper surface of the upper plate 3. These are both well known in the art. The pad is held in place by the edges of the cover cloth 5 which encompass the peripheral edges of the upper plate 3. The buck 1 is mounted in an elevated position on supports S which are in turn mounted on base B, or the floor surface.

Communicating with chamber 2 through the bottom of the lower buck 1 is a steam inlet conduit 8. The end of conduit 8 is connected to a control valve 9 and control valve 9 is connected to steam supply conduit 10 which leads from steam source 11. Valve 9 may be selectively operated to supply steam to chamber 2 of the buck 1. Such valves are believed to be of common construction well known in the art.

Steam source 11 supplies steam under pressure to chamber 2, and valve 9 is controlled by foot pedal 12 at the front of buck 1 and linkage 13, to open and close the communication between buck 1 and steam source 11. The steam supplied from steam source 11 is controlled in pressure and temperature, and can be regulated as necessary.

Heating unit 15 is connected to the underside of lower buck 1 and includes valve housing 16 and heating ducts 17, 18, 19 and 20. Each duct 17-20 communicates at one of its ends through housing ports with housing 16 and at the other of its ends through chamber ports with chamber 2 of buck 1. Ducts 17-20 are arranged so that their points of communication with chamber 2 are spaced from one another.

Valve housing 16 defines entrance ports 22 in its lower wall, and valve elements 23 are urged over ports 22 by springs 24, to close the ports. Springs 24 are weak and function primarily to guide valve elements 23 to their closed position.

Heating elements, such as elements 29 and 30, are positioned in each heating duct 17-20, respectively. Each heating element is electrically connected in parallel to bus lines 31 and 32, line 32 having adjustable control rheostat 33 to control the heat output of the heaters. On-off switch 34 in line 31 controls energization of the heaters. Air heated by the heating elements is raised to a temperature so that after it passes into chamber 2 and through pad 6 and cover 5 it retains the temperature as required by the particular garment fabric for permanent pressing. The heating elements may include electrical resistance type heaters, gas-fired heaters, steam heat exchanges, and the like; however, electrical resistance heaters have been discovered as the least expensive, safe to control, and space saving.

Head 36 is movably supported above the buck 1 by means of arm A which is pivotally connected to buck 1. Head 36 includes a vacuum chamber 38 and a pressing surface 39. The pressing surface 39 is fabricated of a highly porous flexible material such as wire mesh. The wire mesh is preferably of the type having very small openings and an unevenly textured surface. The pressing surface 39 may comprise one or more layers of wire mesh which provide a flexible pressing surface having sufficient

strength to hold a garment and prevent creeping of a garment on the buck as well as being able to exert adequate pressure on the fabric of the garment as may be required for imparting a permanent press.

Use of wire mesh having an uneven surface texture is preferred for the reason that the wire mesh does not readily retain heat nor does it crush or flatten the fabric during application of reasonable pressure so as to produce a "shine" on the garments. Moreover, since each strand of the wire mesh is of small diameter the pressing surface 39 does not tend to collect moisture or mark the garment when the pressing surface is in contact therewith. This is an advantageous feature since it is desired to maintain the original texture of the fabric of the garment during the permanent pressing procedure.

Vacuum is drawn in head 36 by means of conduit 40 being connected between head 36 and a vacuum source 41. The vacuum may be controlled in any one of several ways, for example, it may be continuously applied to the head 10 at all times, or it may be applied to the head only when the head is in pressing relationship with buck 1. The latter application of vacuum to the head may include a control switch which is activated by the arm A or it may be connected to foot pedal 12 controlled by the press operator. All of these arrangements are believed well known in the art and therefore need no further explanation; however, in practical use of the invention, the continuous application of a vacuum to head 36 functions to evacuate the hot air surrounding the buck from the vicinity of the press, which makes the pressing operation more comfortable to the operator. Also, the wire mesh is cooled between pressing operations, thereby further reducing the tendency of the press of imparting a shine to the garments.

Head 36 is fabricated from a flexible material, which can include various plastics or metals; however, the present form of the invention utilizes a polystyrene housing of dished or concave configuration, having a base portion 42 and downwardly extending rim, flange or wall portion 43. Polystyrene is an effective insulating material and prevents heat convection through the housing. The screen which forms the pressing surface of the head is stretched across the vacuum chamber 38 and folded about the edge or periphery 44 of the downwardly extending flange portion 43 of the head at 45 and secured thereto by an adhesive.

As is shown in FIGURES 4 and 5, when head 36 is not in engagement with the buck, screen or pressing surface 39 is stretched by the resiliency of head 36 to an almost flat configuration. When garment 46 is placed on the buck, it can be seen that the seams or folds 48 of the garment will bulge upwardly from buck 1 while the remaining portions of the garment will lie substantially flat on the surface of the buck. When head 36 is lowered into engagement with garment 46 and buck 1, screen 39 will conform to the shape of garment 46, which flexes the walls, or flange 43 of head 36 inwardly to compensate for the effective reduction in size of screen 39. Because of the manner in which screen 39 conforms to the shape of the garment, substantially the whole surface of the garment will feel the same pressure or force from head 36, which reduces the tendency of the garment to develop a shine, and the garment will be smoothly "pressed" throughout its entire upper surface by head 36.

It will be noted that the periphery 44 of head 36 engages buck 1 when head 36 is lowered to engage garment 46. Thus, the vacuum drawn in vacuum chamber 38 will be applied to buck 1 with substantially no leakage of air between head 36 and buck 1. Thus, the steam from chamber 2 will be effectively and efficiently drawn through the garment. In order that the vacuum be uniformly applied to the garment, a sheet of porous material 50 is positioned within the confines of head 36, adjacent screen 39. The sheet of material 50 can be made of various substances, including porous rubber, plastics or woven fab-

rics, including flannel. The material is attached at its edges to head 36 so that the vacuum is applied generally uniformly through screen 39. If desired, a mass of resilient material, such as foam rubber, can be inserted into the cavity of head 36. The massed material will function as a cushion for screen 39, to provide the screen with more "body" during the pressing operation. Of course, the mass of material should be porous to allow the passage of steam and air through head 36.

In order to permanently press garments according to the present invention, it is essential that the necessary curing or heat-setting conditions to effect a permanent press be ascertained. As previously pointed out, these conditions will vary according to the particular fabric being pressed. These conditions are usually available from the mill which has produced the fabric from which the garment is made. As a general observation, it is usually required that the garment be held in its desired shape and subjected to a particular temperature range for a specific period of time. Once these conditions have been ascertained the press operator initially adjusts rheostat 33 so as to provide the buck 1 with appropriate temperature conditions for the permanent pressing operation. When the press is operated, the vacuum drawn in head 36 functions to induce the steam or heated air supplied to chamber 2 of buck 1 to be drawn through the padding of the buck and the garment placed thereon. The heating elements are controlled so that they heat the air drawn through heating ducts 17-20 by the vacuum to a temperature suitable for the fabric. The garment to be permanently pressed is positioned on the upper surface of the pad covering the buck 1 and head 36 is pivoted down into contact with the garment which places the garment under sufficient pressure between the head 36 and the buck 1 to prevent creeping of the garment on the pad. This pressure is, of course, insufficient to cause "shine" on the garment. As the screen 39 engages the garment, it flexes to conform to the shape of the garment, which causes the walls of head 36 to draw inwardly slightly. The periphery 44 of the head engages buck 1 and virtually seals the upper surface of buck 1 to head 36. Steam is introduced to the chamber 2 of the buck 1 through the conduit 10 by manipulation of pedal 12. When the steam enters chamber 2 it engages baffle plate 14 (FIGURE 3) and quickly diffuses throughout the chamber 2 and passes upward through the plurality of openings 4 in the upper plate 3 of the buck, through the pad and into the garment which is to be permanently pressed. A vacuum is immediately applied to chamber 2 of buck 1 as head 36 engages the buck. As a result, the steam supplied to chamber 2 is continuously drawn through the garment and into the chamber 38 of the head and exhausted by way of conduit 40.

Steam pressing of the garment in this manner dampens and loosens the threads of the fabric and thus aids in forming the garment into its desired shape for permanent pressing.

The application of vacuum to the chamber 38 of head 36 while steam is being applied to the garment from the chamber 2 of the buck 1 not only functions to draw the steam through the garment but insures that the work area of the press operator will not become uncomfortable or hazardous because of the presence of excess free steam. The steam is contained by the pad and the garment until it passes through the garment, whereafter it is immediately drawn into the head 36 and therefore cannot escape to the surrounding region. Moreover, the application of the vacuum while steam is being applied to the garment also prevents excess moisture from collecting in the fabric of the garment. This improves the quality of the pressing and makes later drying of the garment less difficult.

After the garment has been steam pressed and while the press is still closed, heated air is directed to the

pressing surfaces. Pedal 12 is released by the operator, which closes valve 9 and terminates the flow of steam into chamber 2. Since a vacuum is still being drawn by head 36, valves 23 in valve housing 16 open to admit air to chamber 2. As the air passes through heating ducts 17-20 and over the heating elements, it is heated to a temperature slightly above that necessary to cure or permanently press the fabric being treated. As the heated air enters chamber 2 it displaces the steam previously admitted to chamber 2 and passes through the garment. Of course, there is a slight heat loss as the heated air approaches the garment, so that the air is at the proper temperature to permanently press the garment as it passes through the garment. The garment may be subjected to the heated air for any necessary period of time to produce curing of the finish or heat-setting of the synthetic fibers. As is apparent, the heated air will pick up a certain amount of moisture in the garment remaining from the steam pressing operation and exhaust it through the vacuum system of the head.

If desired, cooling air may thereafter be supplied to the pressing surfaces for cooling the permanently pressed garment to complete the curing of the fabric. This may be done by providing a separate entry conduit to chamber 2, and closing valves 23 so that atmospheric air passes into chamber 2; however, in practical use of the invention, it has been found that the garments are substantially cured or permanently pressed at the end of the heating cycle and a cooling cycle is not necessary and merely functions to prolong the operation.

Generally, permanent pressing operations may be carried out in connection with the method and apparatus of the present invention by employing a specified pressing temperature range within the range of 250° F. to 450° F. for specified period of time which may vary from a few seconds up to about 20 minutes.

By way of specific example, the present invention may be used to permanently press a polyester/cotton garment by post-curing procedures employing the following general heated air temperature conditions and pressing times:

| °F.: | Minutes |
|------|---------|
| 370  | 2       |
| 340  | 4       |
| 320  | 8       |
| 300  | 15      |

Another example of permanent pressing according to the present invention, but using the re-cure procedure, involves pressing at approximately 325° F. for a period of time in the range of about 25 seconds to 3 minutes.

A further example of permanent pressing according to the present invention and using heat-setting procedures on a polyester/acrylic garment involve pressing at approximately 250° F. for about 15 seconds.

Thus, it may be seen that the apparatus of the present invention is capable of providing a variety of temperature and time conditions as are necessary to perform any particular type of permanent pressing operation. Moreover, these temperature conditions are able to be controlled in such a manner as to prevent overheating of the pressing surfaces thereby preventing possible interference with the permanent pressing operation and damage to the garment. As previously pointed out, this feature is provided by controlled addition of heated air to the pressing surfaces through only the buck in combination with vacuum applied by the head to continuously provide circulation through the garment while it is being permanently pressed. In this manner heat does not tend to build up on the pressing surfaces of the garment. The overall result produced by the method and apparatus of the present invention is a uniformly permanently pressed garment.

It is also pointed out that convenient permanent pressing operations may be carried out in accordance with the present invention employing low pressure even in the

event that the curing of the garment finish occurs at ambient temperatures, it being merely necessary to adjust the temperature of the heated air.

It should be understood that the present invention is particularly suited to automatic sequencing and timing operations since all pressing operations occur when the head is in pressing engagement with a garment overlying the buck. The sequencing of the operations and the operations themselves may be accomplished by well known apparatus. The present invention may also be adapted to presently existing presses with appropriate changes in the manner in which steam, heated air and vacuum are applied. While a foot pedal and rheostat have been illustrated as controlling the steam flow and air temperature, it should be obvious that various other devices can be utilized as well. For instance, a time controlled steam valve and thermostat can be substituted for these elements.

While the disclosed apparatus has been set forth as performing the steaming and heating steps for permanently pressing garments, it should be understood that the apparatus can be utilized to perform the "ironing" function without the "steaming" step. The air can be heated to a temperature high enough to cure a heat setting garment or to a lower temperature when the apparatus is utilized to merely iron or press a garment, whether the garment is a permanent press garment or non-permanent press garment.

What is claimed is:

1. Method of permanently pressing a garment manufactured from a fabric including heat settable synthetic fibers comprising the steps of:

- (a) Supporting a garment on at least a portion of a porous buck surface in a configuration into which it is to be pressed;
- (b) Moving a porous, flexible head surface into engagement with the garment and at least a portion of the buck surface, said head surface at least partially conforming to the configuration of the upper surface of the garment when engaging the garment;
- (c) Flowing steam through the buck surface to the garment;
- (d) Withdrawning the steam from the garment by drawing a partial vacuum through the head surface;
- (e) Terminating the flow of steam while continuing to draw a partial vacuum through the head surface;
- (f) Heating air to a temperature of about 250° F. to about 450° F. and passing the heated air through the buck surface to the garment; and
- (g) Withdrawning the heated air from the garment by drawing a partial vacuum through the head surface.

35

40

45

50

2. Method of claim 1 wherein a partial vacuum is drawn continuously through the head surface during the method steps.

3. Method of claim 1 wherein the garment covers less than the entire buck surface and the head surface engages a portion of the uncovered buck surface continuously around the garment.

4. Method of permanently pressing a garment manufactured from a fabric including heat settable synthetic fibers comprising the steps of:

- (a) Moving a porous, flexible head surface into engagement with at least a portion of a buck surface which has a garment supported thereon, said head surface at least partially conforming to the configuration of the exposed areas of the garment when engaging the garment;
- (b) Drawing a partial vacuum through the head surface continuously during the performance of the method;
- (c) Flowing steam through the buck surface to the garment to be subsequently withdrawn from the garment through the head surface; and
- (d) Terminating the flow of steam through the buck surface while continuing to draw a partial vacuum through the head surface, thus, drawing heated air through the buck surface to the garment to be subsequently withdrawn from the garment through the head surface, said heated air being at a temperature of about 250° F. to about 450° F.

5. Method of claim 4 wherein the garment covers less than the entire buck surface and the head surface engages a portion of the uncovered buck surface continuously around the garment.

#### References Cited

##### UNITED STATES PATENTS

|           |        |                |       |       |
|-----------|--------|----------------|-------|-------|
| 1,544,539 | 6/1925 | Eshelman       | ----- | 38—16 |
| 1,755,488 | 4/1930 | Parizot        | ----- | 38—16 |
| 1,817,406 | 8/1931 | Braun          | ----- | 38—15 |
| 2,644,254 | 7/1953 | Schultz        | ----- | 38—15 |
| 2,703,939 | 3/1955 | Clarke         | ----- | 38—41 |
| 2,784,509 | 3/1957 | Ketchum et al. | ----- | 38—15 |
| 3,025,621 | 3/1962 | Paulsen        | ----- | 38—15 |
| 3,193,952 | 7/1965 | Schlemon       | ----- | 38—15 |

MERVIN STEIN, Primary Examiner

GEORGE V. LARKIN, Assistant Examiner